

## UNITED STATES PATENT OFFICE

2,289,996

PROCESS OF SEPARATING CHALCOPYRITE  
ORES

Anderson W. Ralston and Ervin W. Segebrecht,  
Chicago, Ill., assignors to Armour and Com-  
pany, Chicago, Ill., a corporation of Illinois

No Drawing. Application November 13, 1939,  
Serial No. 304,267

3 Claims. (Cl. 209—166)

This invention relates to the recovery of copper pyrites from ores containing the same, and it comprises processes wherein such ores are subjected to froth flotation in the presence of primary aliphatic amines having from twelve to eighteen carbon atoms and water-soluble salts thereof.

Chalcopyrite ores contain copper as a double sulfide of copper and iron. In addition to the valuable copper and iron constituents much silica in the form of quartz is found in the ore. At the present time these chalcopyrite ores, and by that we mean any ore containing double sulfide of copper and iron, are subjected to froth flotation for the separation of the copper constituents. Many different flotation agents have been proposed for effecting this separation. Many of them, however, are quite expensive, relatively large amounts of costly complex organic compounds being required. What is desired in the art is a flotation agent which can be used under all conditions of acidity or alkalinity in the aqueous slurry of ore pulp, which will not be expensive on a cost-per-ton basis, and which is readily available. We have now discovered that primary aliphatic amines having from twelve to eighteen carbon atoms, as well as amine salts thereof, are highly effective agents for performing this separation. We have discovered that only very small quantities of these agents are required in contrast to much larger amounts of other flotation agents hitherto proposed. Moreover, we have discovered that both the amines as such and their corresponding water-soluble salts are effective. The importance of this is that the flotation can be performed successfully regardless of the acidity or alkalinity of the ore pulp. Consequently, we need not so control the pH value of the pulp that is on the alkaline side or the acid side, as conditions might dictate.

Although the amine salts have been suggested as flotation agents for the separation of phosphate ores and other non-sulfide ores, we are not aware that these agents have been hitherto proposed for the separation of the specific ore of which the present invention is concerned. In our copending application filed of even date herewith, we describe the use of primary aliphatic amine salts as flotation agents for the separation of copper sulfide from ores containing the same. But, as pointed out in that application, the amine salts are very much more effective than the corresponding amines. In the present application we have discovered that the

amines, as well as their salts are highly effective. On the other hand, the primary amines alone are very much better agents for the froth flotation separation of phosphate ores. When phosphate ores are floated with amines the silica appears in the concentrate and the phosphate values in the tailings. When chalcopyrite is subjected to flotation it is the chalcopyrite which appears in the concentrate and the silica in the tailings. Thus each and every ore behaves differently when subjected to froth flotation in the presence of a primary aliphatic amine or its corresponding water-soluble salt, and no predictions can be made with respect to the behavior of one ore from the behavior of another. We emphasize this point so that it may be understood that insofar as the amines and their salts are used as flotation agents, whether they are commercially suitable with respect to cost, and what constituent in the ore floats, can only be determined by experiment and cannot be predicted in advance.

In the present invention we have discovered that both the primary amines and the corresponding water-soluble salts are effective, and each causes commercially practical amounts of the copper-iron sulfide to be concentrated in the concentrate.

All those primary aliphatic amines, and water-soluble salts thereof, which have twelve or more carbon atoms are operative. We can, for example, use dodecylamine, tetradecylamine, hexadecylamine and octadecylamine, as well as their water-soluble salts. Such water-soluble salts are usually the hydrochloride or the acetate. Mixtures of such amines can, of course, be used, as well as mixtures of the amines with the amine salts. One of the most suitable mixtures is that obtained from the reduction of fatty acid nitriles containing twelve or more carbon atoms. Such nitriles can be readily prepared by reacting mixtures of fatty acids with ammonia, and the mixtures of fatty acids can in turn be obtained from any of the common fats by saponification and recovery of the fatty acids from the corresponding soaps.

For purposes of illustration we shall describe our invention with particular reference to the use of dodecylamine and dodecylamine acetate. This amine is readily obtained from the corresponding fatty acid.

The ore used had the following analysis:  $\text{SiO}_2$  48.11%, copper 12.01%, iron 17.51%. The ore was ground and admixed with water in the usual way to form a pulp. This pulp was charged

into a flotation cell filled with water and the suspension adjusted to a pH of 8.1 by the addition of sodium hydroxide. Dodecylamine, in the amount equivalent to 0.05 pound per ton of ore was then added and the mixture subjected to froth flotation. The ore used amounted to 494.65 parts by weight. After flotation a concentrate amounting to 252.26 parts by weight was obtained. This concentrate analyzed as follows:  $\text{SiO}_2$  7.30%, Cu 24.50% and Fe 31.00%. The tailings amounted to 252.39 parts by weight and analyzed as follows:  $\text{SiO}_2$  87.30%, Cu 2.33% and Fe 4.56%.

From this data it is apparent that 98.57% of the silica appeared in the tailings and 7.44% in the concentrate, 90.7% of the copper appeared in the concentrate and 9.03% in the tailings and 86.72% of the iron appeared in the concentrate with 13.28% in the tailings. This gives a copper recovery of 90.97%, an iron recovery of 86.72% and a selectivity co-efficient of 28.3.

Of special interest is the very small amount of primary amine used. We know of no separation hitherto practised on chalcopyrite which uses so little flotation agent.

We shall now give an example using dodecylamine acetate as a flotation agent. In this case the chalcopyrite ore analyzed 49.61% of silica as  $\text{SiO}_2$ , 15.21% of copper and 17.15% of iron. The flotation cell was charged with 498.24 parts by weight of this ore, the cell filled with water and the mixture stirred. 0.30 pound of dodecylamine acetate per ton of ore was then added and the pH adjusted to 5.2. After performing the frothing step we obtained a concentrate amounting to 240.82 parts by weight and a tailing amounting to 257.42 parts by weight. The concentrate analyzed:  $\text{SiO}_2$  0.00%, Cu 29.20% and Fe 34.02%. The tailings analyzed: 96.00% of silica, 0.64% of copper and 1.36% of iron.

On this basis all of the silica appeared in the tailings and none in the concentrate, 97.42% of the copper appeared in the concentrate and 2.58% in the tailings, and 95.91% of the iron 5 appeared in the concentrate and 4.09% in the tailings. This gives a copper recovery of 97.42% and an iron recovery of 95.91%. The selectivity index is, therefore, infinity since no silica appears in the concentrate.

10 From the foregoing results, which can be duplicated when other primary amines and water-soluble salts having six or more carbon atoms are used, it is apparent that these flotation agents are highly effective when only small amounts thereof are used. Although more of the agent can be added to the slurry of ore such is wasteful.

15 We have not described the flotation step in detail since that is well known to those skilled in the art. Our invention is primarily concerned with the use of the aforesaid flotation agents for the separation of chalcopyrite from ores containing the same.

20 Having thus described our invention, what we claims is:

- 25 1. In the froth flotation of copper iron sulfide from ores containing the same the step which comprises subjecting the ore to froth flotation in the presence of a flotation reagent consisting of at least one primary amine compound chosen from the group consisting of primary aliphatic amines having at least twelve carbon atoms and water-soluble salts thereof.
- 30 2. The process as in claim 1 wherein the flotation agent comprises dodecylamine.
- 35 3. The process as in claim 1 wherein the flotation agent comprises dodecylamine acetate.

ANDERSON W. RALSTON.  
ERVIN W. SEGEBRECHT.